

J. M. IRWIN.

PROCESS AND APPARATUS FOR REDUCING COTTON STALKS TO PULP SUITABLE FOR THE  
MANUFACTURE OF PAPER.

APPLICATION FILED SEPT. 14, 1916.

1,250,106.

Patented Dec. 11, 1917.



# UNITED STATES PATENT OFFICE.

JESSE M. IRWIN, OF DALLAS, TEXAS.

## PROCESS AND APPARATUS FOR REDUCING COTTON-STALKS TO PULP SUITABLE FOR THE MANUFACTURE OF PAPER.

1,250,106.

Specification of Letters Patent. Patented Dec. 11, 1917.

Application filed September 14, 1916. Serial No. 120,020.

To all whom it may concern:

Be it known that I, JESSE M. IRWIN, a citizen of the United States of America, residing at Dallas, in the county of Dallas,

5 State of Texas, have invented certain new and useful Improvements in Processes and Apparatus for Reducing Cotton-Stalks to Pulp Suitable for the Manufacture of Paper, of which the following is a specification.

10 This invention relates to new, useful and effective processes and methods for reducing, drawing out and extracting the fibers from vegetable matter and tissues, and particularly it is a process for reducing cotton stalks to pulp suitable for the manufacture of paper, and for such other and further uses to which vegetable pulp may be put.

The object of this invention is to provide a process and method which will combine in 20 comparatively few or a single working operation the different stages which have been necessary to properly reduce vegetable matter to pulp.

Upon information gained through extensive experimentation it is found that the useful vegetable fiber of the cotton stalk can best be drawn out by a combination of mechanical and chemical operations. This invention contemplates such combined use of 30 the two means in a single operation to effectively reduce cotton stalks to a fiber or pulp.

One form of such mechanical means is illustrated herewith and forms an illustrative part of these Letters Patent, said illustrations being given of the machine to aid in a comprehensible understanding of the methods of pulp reduction as herein set out in the appended claims.

40 Previous to the development of the description of the methods and processes hereinafter described, a description of the pulp reducer or digester will be given.

In the drawing Figure 1 illustrates a 45 longitudinal vertical sectional view of the mechanical digester used in connection with the process.

Fig. 2 is a cross sectional view taken upon the line 2—2 of Fig. 1.

50 Fig. 3 is a diagrammatical illustration of correlated crushers or digesters provided upon the reducing apparatus.

Fig. 4 is a diagrammatical view showing

the digester elements of Fig. 3 in an advanced moving position as compared to 55 Fig. 3.

Referring now more particularly to the drawings forming part of the Letters Patent, wherein the same reference characters designate the same parts in the several views, the numeral 1 points out a substantially large reducing or digester boiler. The digester boiler is of a size best calculated to hold and reduce a predetermined quantity of cotton stalks, the diameter and length of 60 same being so designed as to obtain the most efficient working results. The interior of the digester boiler or cylinder will preferably be bored or ground which will give the interior a form of a perfect cylinder 65 adaptable to receive close fitting moving mechanical digester elements. The outer shell or boiler 2 is provided on the digester boiler and has connection with the steam pipe 3 provided with a control valve 4. The steam 70 pipe connects with any suitable source of supply sufficient to raise the temperature of the annular space formed by the outer shell to a high degree or boiling point. Pipe connections 5 are provided and open 75 into the boiler at each end thereof, said pipes are joined and have a common connection with pipe lines 6, 7, and 8, which pipe lines are each provided with a hand valve 9, adaptable to either allow the liquid, contained in the supply with which the said 80 pipe lines connect, to pass into the boiler or withhold it therefrom. A substantially large screw plug 10 and 12 are provided in one head of the boiler, the plug 10 being of 85 sufficient size to admit of the introduction of cotton stalks or vegetable matter to be reduced into the boiler, the screw plug 12 being provided to draw off the pulp. A substantially large drain pipe 13 enters the 90 lower portion of the boiler and is adapted to be used in drawing off the several and various liquids which will be used in connection with the reduction process carried on within the boiler, said pipe being provided 95 with a cut off valve 14.

A substantially large and strong screw-threaded shaft 15 is arranged in the boiler and fixed in an immovable relation to its points of support. A digester wheel 16 105 with an integral extended hub 17 is screw-

threaded upon the shaft and adapted to be revolved thereupon by means hereinafter described. A companion digester wheel 16<sup>a</sup> is provided and has an axis of rotation 5 common to the first named digester wheel and adapted to be run in substantially close contact with the first named wheel. The two digester wheels as illustrated are similar in design and construction, each provided with a central hub as illustrated from 10 which radiate integrally formed webs or blades 18, which webs integrally connect with the rim 19 of the wheel. The function of the digester wheels and blades thereof is 15 to attack and reduce cotton stalks contained in the reduction boiler to pulp by catching the stalks and limbs thereof between the webs or blades and subjecting them to a crushing, rolling and drawing out operation. It will here be understood that the 20 digester wheels are adapted to revolve in opposite directions which permits the webs or blades of the digester wheels to pass one by the other in close relationship. The forward advancing edges of the webs are flared 25 out as indicated in the diagrammatical views Figs. 3 and 4. The following edges of the webs gradually turn inwardly in a curvilinear form until the edge of the rim 30 of the wheel is approximately reached where the remaining portion of the said web is formed in a parallel relation with the plane of the rim of the wheel. This brings the following rear portions of the 35 webs into a close relationship one with the other, and into such a close passing position as to admit only very small vegetable fibers to pass therebetween. Said following rear portions of the webs may be termed the 40 working faces or portions of the webs, which working faces of the webs as later seen will attack and by attrition roll, crush, reduce and draw out the fiber from the cotton stalk.

45 A substantially large and heavy shaft 20 has one extremity fixed in the head of the boiler and in contact with the extremity of the screw-threaded shaft, a pin 21 being employed to fix them one to the other in an 50 immovable relation. A tubular shaft 22 is provided and journaled upon the shaft 20, said tubular shaft passing through the head of the boiler and having its inner extremity lying in contact with the extended hub of 55 the wheel 16. A screw-threaded connecting sleeve 23 is provided and adapted to join in a fixed relation the tubular shaft with the wheel 16 in such a way that said wheel may be driven in revolution by the tubular shaft 60 22. A tubular shaft 24 is confined on first named shaft and journaled on its inner extremity upon the connecting sleeve 23, and journaled upon its outer extremity on a bearing 24, the members 23 and 24 serving 65 to support the shaft 24 in journaled relation

upon the shaft 22. The second named wheel is fixed upon the shaft 24 and adapted to be driven in revolution by said shaft.

A motor 25 is movably arranged upon the shaft 20, the base of said motor being so arranged as to allow the motor to slowly move along in an upright position the length of the shaft. Said shaft is provided with a groove or channel extending the entire length thereof. The motor base which 75 is confined upon the shaft is provided with a rib which lies within and engages the walls of the channel, holding said motor in a vertical and upright position. Gears 26 and 27 are fixed upon the motor shaft. A 80 reverse gear 28 is carried by a stud fixed to the motor base. A gear 29 is fixed to the extremity of the tubular shaft 22 and engages the reverse gear 28. A gear 30 is fixed to the shaft 24 and engages the gear 26. 85 The means of transmission, as just described, with the gear 28 interposed between the motor and the shaft allows the shafts to be driven in an opposite direction which carries the digester wheels in an opposite 90 direction one from the other. A thrust-bearing 31 is confined upon the shaft 22 and interposes between the gear 29 and extremity of the shaft 24.

The motor during the operation will 95 drive the two shafts in an opposite direction one from the other, the shaft 22 driving the wheel 16 and moving it along the screw-threaded shaft 16 causing said wheel to travel along the length of the boiler as 100 said wheel revolves. Through the agency of the thrust-bearing 31 interposed between the gear 29 and tubular shaft 24 the correlated second named digester wheel will be confined to the same longitudinal travel and 105 speed as wheel 16 is undergoing. The assembly and arrangement of the mechanical digester as described provides a pair of correlated oppositely revolving longitudinally traveling digester wheels adapted to 110 revolve with their peripheries in close contact with the inner walls of the cylindrical boiler.

Figs. 3 and 4 are diagrams illustrative of different and varying operating positions 115 to the webs or blades of the digester wheels. Fig. 3 shows the oppositely traveling webs or blades as indicated by the arrows and the following rear working faces of said blades approaching each other. Fig. 4 illustrates the correlated working webs or blades in their opposite direction of travel as indicated by the arrows and with the following or trailing working faces passing each other in very close relation one with the other.

The digester wheels are adapted to be driven at a substantially slow speed ranging from one hundred to three hundred revolutions per minute which will cause the entire assemblage of the bearing transmis- 125 130

sion arrangement herein disclosed to travel along the shafts. Owing to the slight pitch of the thread upon the shaft the digester wheels will require considerable time in 5 traveling from one extremity of the boiler to the other. At the time the digester wheels have reached the end of the boiler it will be necessary for an attendant operator to reverse the current through the motor 10 and start the correlated digester wheels in the opposite direction. This operation is continual throughout the period of work 15 upon the stalks contained in the digester, means being provided if desirable for some form of automatic control for reversing the current in the motor and the direction of operation of digester wheels at the end of each period of travel.

A description will now be given of the reduction process which includes the introduction of certain chemical reducing and dissolving agents into the boiler with the mass. The cotton stalks will be harvested and introduced into the digester boiler through the 25 plug 10. The boiler will be filled with said stalks and the machine set in operation, at the same time the water supply pipe line 6 will be opened allowing water to flow through the pipes 5 into each end of the 30 boiler. The tremendous agitation and attrition set up on the interior of the boiler by the operation of the oppositely revolving digester wheels will thoroughly wash and cleanse the stalks of any dirt or foreign matter 35 which may have been included as the stalks were placed into the reduction boiler. After a sufficient washing process is carried on the water pipe line is closed and all the water allowed to drain from the boiler 40 through the conduit 13.

With the digester wheels in continuous operation the pipe line 7 is opened which admits to the boiler the flow of cooking liquor or reducing liquid. The pipe line 7 connects with any suitable reservoir which holds in storage and in reserve a quantity of previously prepared cooking liquor or stalk reducing liquid, which liquid is a chemical solution consisting of any strong 50 alkaline or caustic preparation. Preferably a preparation of potassium hydroxid or caustic potash in the per cent. of about one tenth, thoroughly mixed with water, will be used in the mechanical digester in connection with the reduction. After the cooking 55 is introduced into the digester boiler and the revolving digester wheels have been in continual operation for a considerable period of time the stalks will be rolled, mashed and drawn and by the continual attrition of the coöperating blades of the wheels and by the chemical attacks of the reducing liquid upon the stalks the same will begin to take on a semi liquid condition 60 until the whole mass contained in the boiler

will be reduced to a homogeneous plastic semi fluid pulp.

During this operation as described steam can be used to advantage and further assist and hasten the disintegration and reduction 70 of the stalks by admitting steam to the boiler and keeping the cooking liquor to a very high temperature. Steam may also be admitted to the annular steam chamber contained between the boiler and the outer shell, 75 this will raise the temperature of the boiler to a high degree and keep the cooking liquor and reduction liquor very hot. After the stalks are thoroughly reduced and all the fiber of said stalks are drawn and divided 80 and disintegration is thorough, the steam and cooking liquor pipe lines will be closed and the water pipe line again opened at which time the large drainage conduit 13 will also be opened.

The strainer devices contained in the head of the conduit 13 will prevent the mass of pulp from flowing from the boiler to allow the water and cooking liquor to pass out freely. With the digester wheels in continual 85 operation the fresh water supply will be turned into the digester boiler. The water will be ready to run and mingle with the reduced pulp until the cooking liquor has been thoroughly washed therefrom which 90 will leave the mass inside the boiler a clean pulp free from cooking liquor and free from the caustic and aciduous solutions.

The pipe line 8 having connection with the pipe lines 5 also has direct connection 100 with a reservoir or storage tank not shown. Said storage tank is provided to contain suitable bleaching liquids and preparations which may be used to bleach whiten and further prepare the pulp for commercial 105 paper making. After the washing process is thoroughly completed and the water drawn from the digester boiler the bleaching liquid pipe line 8 will be opened and a certain quantity of bleaching chemicals introduced 110 into the boiler, while the digester wheels are in continued operation. After the bleaching operation is thoroughly complete and the mass is whitened to a desired degree the operation of the digester apparatus will be 115 discontinued and the pulp drawn from the digester boiler through the plug 12.

The design of the two correlated digester wheels with their coöordinated attrition blades or webs is such that a space or opening is left between the blades of the wheels when said blades or webs are registered one with the other, or when one blade is directly behind the other. At this period of the travel of the wheels it would seem that 120 a considerable quantity of stalks or pulp would escape or pass unground by the wheel. But the advancing curvilinear design of the blade and its outwardly projecting contour in respect to its advance of travel will in 125 130

fact pass forward and scoop or pick up and throw back any quantity of stalks or un-reduced pulp toward the first wheel. The blades of the first wheel will immediately 5 catch the stalks or pulp and cause same to be confined in the press formed between said blades and as the movement of the blades continue the pulp will be gathered closer and closer in between the diminishing 10 space formed between the blades and will be rolled and ground and reduced by friction to fibrous matter. As the pulp is reduced to a very fine texture and dissolved into a semi-liquid and homogeneous state, 15 it will be so fine in texture that the wheels will no longer catch it and confine it there-between but will allow the reduced mass to squeeze and run by the blades of the wheel.

When the digester wheels start in their 20 movement from one end of the cylinder to the other a considerable pressure will be exerted on the mass in front of the forwardly advancing digester wheels. This pressure is set up by the positive drive along the 25 screw-threaded shaft of the said digester wheels, which pressure will cause the mass of matter in front of the wheels to be pressed into the revolving blades. The revolving blades will have a tendency to some extent to 30 cause the mass in the boiler to revolve, which movement on the part of the unreduced mass will not effect the passage of the unreduced stalks and pulp into the wheels since the pressure on the mass generated by the wheels 35 will be sufficient to project same into the blades.

The tremendous heat set up in the reducing boiler through the agency of steam combined with the disintegrating and attacking 40 capacity of the reducing liquids combined with the tremendous and vigorous attrite movements of the oppositely revolving wheel will thoroughly and effectively break up, reduce, divide, disintegrate and draw 45 out the fiber of the cotton stalks leaving the mass of pulp consisting of a fiber of considerable tensile strength and length, which fiber when manufactured into paper 50 will have a high degree of tensile strength and interior cohesion.

The process and methods herein disclosed to be used in connection with the reduction of cotton stalks to commercial pulp is presented to include those variations and 55 changes in degree of operation which hereinafter may be resorted to in obtaining similar results when such variations are construed to come within the meaning of the following claims:

60 1. In a process for the reduction of cotton stalks to pulp, the initial step of placing the cotton stalks in a container, the hydration of the stalk mass, then subjecting the mass to

chemical action, and the mass alternately compressed first from one end of the container then from the other, during which alternate compressing periods the individual stalks and fiber body of the mass are caused to pass through and between moving interstices of the container setting up such a frictional engagement between the stalk or fiber body and the machine element as to cause the tentacles and fiber to be drawn and abstracted from the body of the stalk.

2. In a pulp reducing machine for the purpose of reducing plant growth to pulp suitable for the manufacture of paper, the combination with a cylindrical boiler container, a shaft axially arranged in the container, and a plurality of revolving attrition wheels mounted on the shaft adapted to travel among the mass of plant growth reducing same to pulp.

3. In a pulp reducing machine, the combination with a boiler container, of a shaft 85 axially arranged in the container, a pair of bladed grinding wheels mounted upon the shaft and adapted to travel along the shaft from end to end simultaneously as said wheels are in a motion of revolution. 90

4. In a pulp reducing machine, the combination of a cylindrical container, of a screw threaded shaft fixed in the container, a pair of bladed attrition or grinding wheels carried upon the screw threaded shaft and 95 adapted to travel along the threads of the shaft and among the mass of matter to be reduced.

5. In a pulp reducing machine of the character described, the combination with 100 a steaming and cooking boiler wherein the mass of material to be reduced may be steamed, hydrated and cooked in one and the same container, of a plurality of bladed attrition wheels arranged in a contiguous 105 relation one with another adapted to pass back and through the mass to be reduced in such a manner that frictional engagement is set up between the several attrition wheels as the mass is forced through the 110 contiguous blades of the said wheels.

6. In a pulp reducing machine, the combination with a container used for the purpose of hydrating, steaming and cooking the mass, of a shaft axially arranged in the 115 container, of two attrition wheels provided with oppositely turned blades carried upon the shaft and adapted to travel along the shaft contiguously one with the other and revolving in opposite directions.

In testimony whereof I affix my signature in the presence of two witnesses.

JESSE M. IRWIN.

Witnesses:

V. R. SANDERS,  
J. C. LEDBETTER.